

June 9, 1953

G. MOHLING ET AL

2,641,540

FERROUS BASE CHROMIUM-NICKEL-TITANIUM ALLOY

Filed July 19, 1951

5 Sheets-Sheet 1

OUR ALLOY - HEAT NO. 43297  
EFFECT OF SOLUTION TEMPERATURE ON  
STANDARD AND V-NOTCH RUPTURE STRENGTH  
AND RUPTURE DUCTILITY  
TESTS AT 1200° F. - 60,000 P.S.I.



HEAT TREATMENT:  
SOLUTION TEMP. - 1 HR. OIL  
+ 1325° F. - 16 HOURS AIR

*Fig. 1*

INVENTORS  
Gunther Mohling  
Wasil W. Dyrkacz  
BY  
Green, McCallister, Miller  
THEIR ATTORNEYS

June 9, 1953

G. MOHLING ET AL

2,641,540

FERROUS BASE CHROMIUM-NICKEL-TITANIUM ALLOY

Filed July 19, 1951

5 Sheets-Sheet 2

EFFECT OF TITANIUM CONTENT ON V-NOTCH  
RUPTURE STRENGTH AND RUPTURE DUCTILITY  
[STANDARD TEST]

ALLOY A VS. OUR ALLOY  
TESTS AT 1200°F. - 60,000 P.S.I.



HEAT TREATMENT  
1800°F. - 1 HR. OIL  
1325°F. - 16 HRS. AIR

*Fig. 2*

INVENTORS  
BY  
Gunther Mohling  
Wasil W. Dyrkacz  
Green, McCallister, Miller  
THEIR ATTORNEYS

June 9, 1953

G. MOHLING ET AL

2,641,540

FERROUS BASE CHROMIUM-NICKEL-TITANIUM ALLOY

Filed July 19, 1951

5 Sheets-Sheet 3

OUR ALLOY  
V-NOTCH AND STANDARD RUPTURE STRENGTH  
VS. BRINELL HARDNESS  
TESTS AT 1200° F. - 60,000 P.S.I.



HEAT TREATMENT:  
1800° F. - 1 HR. OIL  
1325° F. - 16 HRS. AIR

*Fig. 3*

INVENTORS  
Gunther Mohling  
Wasil W. Dyrkacz  
BY *Green, McCallister, Miller*  
THEIR ATTORNEYS

June 9, 1953

G. MOHLING ET AL

2,641,540

FERROUS BASE CHROMIUM-NICKEL-TITANIUM ALLOY

Filed July 19, 1951

5 Sheets-Sheet 4

OUR  
ALLOY

Heat 43297

Heat Treatment  
1650° F - 1 hr., Oil Quenched  
plus  
1325° F - 16 hrs., Air Cooled



Fig. 4

A.S.T.M. Grain Size Range - 8 to finer than 8 - Average: Finer than 8

OUR  
ALLOY

Heat 43297

Heat Treatment  
1800° F - 1 hr., Oil Quenched  
plus  
1325° F - 16 hrs., Air Cooled



Fig. 5

A.S.T.M. Grain Size

Range - 5 to finer than 8

Average - 6 to finer than 8

INVENTORS  
Gunther Mohling  
Wasil W. Dyrkacz  
BY Green, Mc Callister, Miller  
THEIR ATTORNEYS

June 9, 1953

G. MOHLING ET AL

2,641,540

FERROUS BASE CHROMIUM-NICKEL-TITANIUM ALLOY

Filed July 19, 1951

5 Sheets-Sheet 5

OUR  
ALLOY

Heat 43297

Heat Treatment  
1900°F - 1 hr., Oil Quenched  
plus  
1325°F - 16 hrs., Air Cooled



*Fig. 6*

A.S.T.M. Grain Size

Range - 2 to 8

Average - 3 to 6

OUR  
ALLOY

Heat 43297

Heat Treatment  
2050°F - 1 hr., Oil Quenched  
plus  
1325°F - 16 hrs., Air Cooled



*Fig. 7*

A.S.T.M. Grain Size

Range - Larger than 1 to 6

Average - Larger than 1 to 3

INVENTORS  
BY *Gunther Mohling*  
*Wasil W. Dyrkacz*  
*Green, McCallister, Miller*  
THEIR ATTORNEYS

## UNITED STATES PATENT OFFICE

2,641,540

## FERROUS BASE CHROMIUM-NICKEL-TITANIUM ALLOY

Gunther Mohling, Loudonville, and Wasil W. Dyrkacz, Newtonville, N. Y., assignors to Allegheny Ludlum Steel Corporation, Brackenridge, Pa., a corporation of Pennsylvania

Application July 19, 1951, Serial No. 237,534

8 Claims. (Cl. 75—128)

1

This invention pertains to ferrous alloys and particularly, to improved austenitic chromium-nickel-titanium ferrous alloys.

Due to recent strides being made in the development of aircraft engines, e. g. jet engines and gas turbines, the need has arisen for new and improved alloys which may be made commercially on a production basis and which will stand up when highly stressed rotating parts are to operate at a temperature of around 1000° to 1350° F. Heretofore, there has been no heat treatable alloy which would fully meet requirements in this respect as to ductility within such a temperature range and which could be produced on a production basis by ordinary arc melting, high tonnage procedure. An alloy of this type for use in rotating parts must not only stand up at such temperatures, but must have other characteristics which will comply with the rather rigid and high requirements of such a utilization.

Heretofore, one type of alloy has been produced which we will hereinafter specify as alloy A that falls within the minimum requirements of such a utilization, except for ductility at the critical (normal embrittlement) temperature of 1000° to 1200° F. to which rotating parts are subjected. Alloy A is thus limited to stationary utilizations as it has an insufficient ductility for rotating parts. Alloy A has the following general composition: small amounts of carbon, silicon, manganese and aluminum, about 30% nickel, 15% chromium and 2.0% titanium. This alloy is a commercial type, but has an extremely short rotating part operating life period, is notch sensitive, and fails suddenly.

Another alloy which will be hereinafter designated as alloy B (see U. S. Patent No. 2,519,406) has been found to generally fulfill the minimum requirements of the subject utilization up to and including operation of the working parts at such temperature, but has only been successfully produced on a pilot plant scale and at a relatively high cost. This latter alloy requires special forging and heat treatment processing and is produced by induction melting. The closely controlled hot-cold forging work ties up forging equipment for long periods of time. We, as well as those skilled in the art, have definitely determined that such an alloy cannot be produced on a large commercial scale by conventional

2

steel making processes and have the requisite properties.

It thus appears that there is a definite and critical need for an improved heat treatable alloy which can be produced in high tonnage and which will have a generally higher ductility at operating temperatures than those now available and which will retain its ductility in the temperature range of 1000°-1200° F. (normal brittle range) and well up to 1350° F. Such temperatures are encountered in ordinary usage of rotating engine parts and thus, the life of such parts is governed by the ductility of the metal. Furthermore, explosion failure which is caused by very brittle characteristics, must be avoided at all costs and if failure is to occur, it must be of a gradual nature, so that steps may be taken to replace the part before its utilization becomes dangerous.

20 It has thus been an object of our invention to provide an improved chromium-nickel-titanium ferrous alloy of an austenitic type which will not only have good forgeability, machinability and an excellent high strength, but will retain its ductility in a moving part utilization and especially, at elevated temperatures of 1000° to 1200° F.

Another object has been to provide a wrought, austenitic, precipitation-hardened alloy which will meet requirements for rotating aircraft engine parts;

30 A further object has been to provide an alloy of this type which can be produced on a commercial production basis and can be simply and inexpensively processed as well as produced;

35 These and many other objects of our invention will appear to those skilled in the art from the further description thereof.

In the drawings, Figures 1 to 3, inclusive, are curves graphically illustrating the improved characteristics of alloys of our invention and Figures 4 to 7, inclusive are photomicrographs showing the effect of various heat treatments on alloys of our invention.

40 In carrying out our invention, we have been able to provide an alloy which has highly superior characteristics under all conditions of utilization, which can be produced by conventional melting practice, whose properties can be developed by heat treatment without special work-

ing and heat treating procedures, and which can be produced relatively inexpensively and processed simply to develop its characteristics. It has a life period far in excess of 1000 hours in rotating engine part utilizations, as based on test data comparisons. It can be hot worked and treated in commercial size heats using standard or conventional equipment. In this alloy, the maximum carbon content is highly critical, and the manganese content provides increased rupture ductility and improved forgeability. Also, vanadium is a highly important and critical element. The alloy permits a higher manganese to silicon ratio. The manganese and vanadium are employed as alloy additions and not as scavengers, as they are introduced directly into the melt and not at the end for cleanup purposes and thus, are essentially in solid solution form in the alloy. The proportioning of vanadium to titanium and molybdenum contents is also highly critical and is believed to constitute the crux of the invention from the standpoint of the specified ranges of chromium, nickel and silicon contents.

In this alloy, although not necessary, cobalt can be added up to 25% to further increase its strength. The element aluminum is generally considered to contribute toward brittleness. We have found that it increases rupture ductility considerably, but at the expense of rupture strength (as evidenced by melt A-416 of Table VI). In our alloy, we have discovered that the adverse effect of a higher aluminum content on rupture strength can be more than offset by the addition of cobalt in amounts up to 25%, e. g. as shown in Table VI, melt A-409 (which contains 1.2% aluminum) is considerably strengthened by the addition of 20% cobalt. The fact that our alloy can take a higher percentage of aluminum is further indicative of its novel characteristics.

Our alloy in its broader aspects contains carbon in relatively low amounts up to .15% maximum, manganese within a range of .50 to 3.00% (not as a scavenger but as an essential alloying element introduced into the solution), silicon up to 1.50%, chromium within a range of about 5 to 22%, nickel within a range of 7 to 50%, titanium within a range of .50 to 3.50%, a relatively low percentage of molybdenum of about .25 to 2.00%, a highly critical percentage of vanadium of .10 to 1.50%, up to 25% cobalt, and up to 2.5% aluminum. In our alloy, the remainder is iron with incidental impurities, such as nitrogen, phosphorus and sulphur.

While in general, increasing the titanium content increases the rupture strength and tensile strength, it also decreases rupture ductility below a useful level when a critical titanium content is reached. In alloy A, this content appears to be about 1.5% titanium, and in alloy B, about 1.9% titanium. In alloys of our invention, useful ductility is maintained up to at least about 3% titanium (see Table IV). This is obtained by proportioning of the other elements and particularly, of the vanadium and molybdenum to offset or reduce the embrittling effect of titanium within the ranges specified. Our alloys, therefore, permit a much higher than ordinary range of titanium, while still insuring high strength combined with good rupture ductility.

The optimum range of our alloy which we have found highly satisfactory consists of carbon in an amount up to .15 maximum, about .5 to 2.0% manganese, about .4 to 1.5% silicon, about 12 to

18% chromium, about 20 to 35% nickel, about 1.0 to 1.5% molybdenum, about .10 to .50% vanadium, and about 1.5 to 2.9% titanium, with aluminum in a maximum amount of 0.35%.

5 A specific alloy which we have produced with optimum results contains about .08 maximum carbon, about 1.0 to 2.0% manganese, about .50 to 1.25% silicon, about 12 to 16% chromium, about 24 to 28% nickel, about 1.0 to 1.5% molybdenum, about .10 to .50% vanadium, about 1.75 to 2.25% titanium, and incidental amounts of aluminum from the addition of ferro-alloys.

15 It will be noted that our alloys save on highly strategic materials and as will hereinafter be shown by test data, are inherently ductile, even at temperatures of about 1200° F., as demonstrated by notched rupture tests. Grain coarsening begins at about 1850° F., see Figures 4 to 7, inclusive. Further, our alloys do not need cold working, since their properties can be developed by a solution treatment and age-hardening (see Figure 5) and they can be handled in melting, forging, and heat treating in the same manner as any commercial alloy.

20 25 Best results are obtained by employing a solution heat treatment of about 1800° F. for one hour and rapidly cooling in a suitable fluid quenching medium (such as oil, air or water), followed by age hardening at about 1325° F. for about 16 hours plus air or furnace cooling (in a gaseous atmosphere). That is, it has been determined that 1800° to 1850° F. is about the highest practical temperature to which the alloy can be raised before grain coarsening sets in and temperatures higher than this, as shown by Table II, produce some gain of strength at the cost of rupture ductility and increased notch sensitivity. Another advantage of our alloys is that a high titanium content can be employed without seriously adversely effecting their ductility, see Table IV. Ductility may be increased by lowering the amount of titanium, but with a greatly reduced rupture strength and tensile strength below about 1.45% titanium. We have found that vanadium is a highly controlling element in offsetting the embrittling tendency of titanium.

25 30 Although with our alloys, better results can be obtained employing any conventional heat treatment, optimum results are obtained by the 1800° F. solution treatment and subsequent age hardening treatment which has been previously discussed.

35 40 As compared to the best alloy available prior to our present invention, namely alloy B (as produced by special procedure), a typical alloy of our invention has a Brinell hardness of 140 to 170 in the solution treated condition, as compared to hardness of 140 to 160 for alloy B, and as solution treated and aged, has an assured hardness of 248 to 341 and higher, as compared to hardness of 248 to 302 for alloy B. It appears that our alloys not only have an increased hardness, strength, etc., but have an increased ductility such that the operating life of working parts can be greatly improved and particularly so, when in operation, they are subjected to heat of up to about 1350° F. and particularly, in the critical range of 1000° to 1200° F. In addition, products made with our alloys can be produced at much lower cost than alloy B, as they do not require special forging and heat treating practice. Center segregation is reduced or eliminated in our alloys when produced in large commercial melts so as to provide material which will have sufficient 45 50 55 60 65 70 75 center ductility in large forgings, such as turbine

rotors. In our alloys, segregation is minimized by limiting the molybdenum content to a 2% maximum.

The V-notch rupture tests as employed herein are an indication of rupture ductility. When high temperature metals of the type herein being con-

an included angle of 60° with a .005 inch radius at the base of the notch.

In the following Table I, we have set forth test data on alloys of our invention on three commercial production heats of 2 and 10 tons made in ingot sizes of 9" to 25" square.

TABLE I

|                                                | Heat 43297 |               | Heat 43300 |               | Heat 62918 |               |
|------------------------------------------------|------------|---------------|------------|---------------|------------|---------------|
|                                                | Hrs.       | Percent Elong | Hrs.       | Percent Elong | Hrs.       | Percent Elong |
| <b>Rupture Tests:</b>                          |            |               |            |               |            |               |
| 1,200° F.—60,000 p. s. i.<br>(standard)        | 147        | 5.4           | 156        | 5.9           | 118        | 7.3           |
| 1,200° F.—60,000 p. s. i.<br>(.005" R-V-Notch) |            |               |            |               | 670        |               |
| 1,200° F.—50,000 p. s. i.<br>(Standard)        |            |               |            |               | 483        | 8.4           |
| 1,300° F.—42,500 p. s. i.<br>(Standard)        |            |               | 188        | 9.5           | 469        | 8.2           |
|                                                |            |               | 207        | 9.4           | 167        | 16.4          |
|                                                |            |               | 210        | 9.6           | 109        | 11.8          |
| <b>Room Temperature Tensile:</b>               |            |               |            |               |            |               |
| .2% Yield Strength                             |            | 103,800       |            | 111,000       |            | 100,800       |
| Tensile Strength                               |            | 157,500       |            | 158,000       |            | 147,000       |
| Percent Elongation                             |            | 25.0          |            | 25.0          |            | 25.0          |
| Percent Reduction                              |            | 38.2          |            | 41.0          |            | 42.5          |

Heat treatment on above:  
1,800° F.—1 hour—oil+  
1,325° F.—16 hours—air.

sidered have a low rupture ductility, the V-notch rupture life is considerably less than the standard rupture life and thus, they are considered to be "notch sensitive." In carrying out this test, we

Table II and the photomicrographs of Figures 4 to 7, inclusive, illustrate the importance of solution heat treatment in developing the structure and properties of our alloys.

TABLE II—OUR ALLOY  
*Effect of solution temperature on standard and V-notch rupture strength, rupture ductility and grain size*

## ANALYSIS

| Heat No. | C   | Mn   | Si  | Cr    | Ni    | Mo   | Ti   | V   | Al  |
|----------|-----|------|-----|-------|-------|------|------|-----|-----|
| 43297    | .03 | 1.21 | .86 | 15.12 | 26.16 | 1.32 | 1.94 | .23 | .40 |

## STRESS RUPTURE AT 1,200° F.—60,000 p. s. i.

| Heat Treatment        | Standard Test    |        |                   | .005" R-V-Notch Test, Hours to Rupture | Grain Size, A. S. T. M. |                    |
|-----------------------|------------------|--------|-------------------|----------------------------------------|-------------------------|--------------------|
|                       | Hours to Rupture | Elong. | Percent Red. Area |                                        | Range                   | Average            |
| 1,650° F.—oil+        | 62               | 9.0    | 12.9              | 240                                    | 8 to finer than 8       | Finer than 8       |
| 1,325° F.—16 hrs.—air | 147              | 5.4    | 9.4               | 145                                    | 5 to finer than 8       | 6 to finer than 8  |
| 1,800° F.—oil+        |                  |        |                   |                                        |                         |                    |
| 1,325° F.—16 hrs.—air | 180              | 2.4    | 4.5               | 3.7                                    | 2 to 8                  | 3 to 6             |
| 1,900° F.—oil+        |                  |        |                   |                                        |                         |                    |
| 1,325° F.—16 hrs.—air | 2,050° F.—oil+   | 95     | 3.0               | 1.5                                    | Larger than 1 to 6      | Larger than 1 to 3 |
| 1,325° F.—16 hrs.—air |                  |        |                   |                                        |                         |                    |

make a notch of .040 inch deep in a .275 inch diameter test bar and the sides of the notch form

Table III sets forth six typical melts of our alloy giving test data as to the same.

7  
TABLE III  
8

| Melt No. | Type of Test | Temp.,<br>° F. | Stress,<br>p. s. i. | Hrs. to<br>Rupture | Percent<br>Elong. | Percent<br>Red. Area |
|----------|--------------|----------------|---------------------|--------------------|-------------------|----------------------|
| A-285    | Std.         | 1,200          | 60,000              | 161                | 5.9               | 11.9                 |
|          | .005" R V-N  | 1,200          | 60,000              | 241                | 8.8               | 16.6                 |
| A-286    | Std.         | 1,200          | 60,000              | 92                 | 8.8               | 16.6                 |
|          | .005" R V-N  | 1,200          | 60,000              | 627                | 10.0              | 16.6                 |
| A-287    | Std.         | 1,200          | 60,000              | 108                | 10.0              | 16.6                 |
|          | .005" R V-N  | 1,200          | 60,000              | 649                | —                 | —                    |
| A-254    | Std.         | 1,200          | 60,000              | 112                | 9.2               | 22.2                 |
|          | .005" R V-N  | 1,200          | 60,000              | 533                | —                 | —                    |
| A-373    | Std.         | 1,200          | 60,000              | 211                | 10.6              | 22.2                 |
|          | .005" R V-N  | 1,200          | 60,000              | 902                | —                 | —                    |
| A-374    | Std.         | 1,300          | 42,500              | 112                | 17.3              | 41.0                 |
|          | .005" R V-N  | 1,200          | 60,000              | 105                | 10.0              | 17.5                 |
| A-374    | Std.         | 1,300          | 42,500              | 538                | —                 | —                    |
|          | .005" R V-N  | 1,300          | 42,500              | 82                 | 15.3              | 33.0                 |

  

| Melt No. | C   | Mn   | Si  | Cr   | Ni   | Mo  | Ti  | V   | Al  |
|----------|-----|------|-----|------|------|-----|-----|-----|-----|
| A-285    | .04 | 1.23 | .81 | 13.9 | 25.9 | 1.3 | 2.0 | .44 | .13 |
| A-286    | .04 | 1.25 | .82 | 14.4 | 26.1 | 1.3 | 1.8 | .32 | .03 |
| A-287    | .06 | 1.23 | .84 | 14.2 | 25.9 | 1.2 | 1.8 | .16 | .07 |
| A-254    | .03 | 1.34 | .71 | 14.1 | 26.4 | 1.0 | 1.8 | .69 | .16 |
| A-373    | .05 | 1.28 | .76 | 14.8 | 26.3 | 1.3 | 1.9 | .35 | .14 |
| A-374    | .04 | 1.14 | .78 | 14.9 | 26.5 | 1.3 | 1.7 | .34 | .16 |

Stress-rupture data on alloy A shows that rupture ductility decreases with an increase in titanium content (see Figure 2). In our alloy, see Table IV and Figure 2, an increase of

ductility. This is true even when hardness is in excess of 290 Brinell which is in contradiction to alloy B. In this connection, attention is called to the data set forth in Table IV and Figure 3.

TABLE IV  
*Effect of increasing Ti content on tensile, hardness and rupture properties*

| Melt No. | Ti  | C   | Mn   | Si   | Cr   | Ni   | Mo  | V   | Al  |
|----------|-----|-----|------|------|------|------|-----|-----|-----|
| A-374    | 1.7 | .04 | 1.14 | .78  | 14.9 | 26.5 | 1.3 | .34 | .16 |
| A-373    | 1.9 | .05 | 1.28 | .76  | 14.8 | 26.3 | 1.3 | .35 | .14 |
| A-371    | 2.5 | .04 | 1.14 | 1.02 | 15.0 | 26.5 | 1.3 | .38 | .10 |
| A-372    | 2.9 | .05 | 1.28 | 1.11 | 14.7 | 26.4 | 1.3 | .39 | .12 |

## RUPTURE PROPERTIES

| Melt  | Type Test   | ° F.  | Stress | Hrs. to<br>Rupture | Percent<br>Elong. | Percent<br>Red.<br>Area | Rock. C.<br>Hardness<br>(after<br>test) |
|-------|-------------|-------|--------|--------------------|-------------------|-------------------------|-----------------------------------------|
| A-374 | Std.        | 1,200 | 60,000 | 105                | 10.0              | 17.5                    | 31                                      |
|       | .005" R V-N | 1,200 | 60,000 | 538                | —                 | —                       | 32                                      |
| A-373 | Std.        | 1,300 | 42,500 | 82                 | 15.3              | 33.0                    | 30                                      |
|       | .005" R V-N | 1,200 | 60,000 | 211                | 10.6              | 22.2                    | 32                                      |
| A-371 | Std.        | 1,200 | 60,000 | 902                | —                 | —                       | 32                                      |
|       | .005" R V-N | 1,300 | 42,500 | 112                | 17.3              | 41.0                    | 36                                      |
| A-372 | Std.        | 1,300 | 42,500 | 225                | 15.0              | 22.0                    | 41                                      |
|       | .005" R V-N | 1,200 | 60,000 | 288                | 11.6              | 19.5                    | 39                                      |
| A-372 | Std.        | 1,300 | 42,500 | 118                | 11.2              | 46.5                    | 35                                      |

## ROOM TEMPERATURE PROPERTIES

| Melt  | 0.2%<br>Yield<br>Strength | Tensile<br>Strength | Percent<br>Elong. | Percent<br>Red. Area | Brinell<br>Hardness |
|-------|---------------------------|---------------------|-------------------|----------------------|---------------------|
| A-374 | 93,600                    | 140,000             | 28.0              | 44.6                 | 269                 |
| A-373 | 96,000                    | 143,500             | 27.0              | 44.0                 | 277                 |
| A-371 | 115,500                   | 163,500             | 24.0              | 34.1                 | 302                 |
| A-372 | 135,000                   | 178,250             | 11.0              | 14.5                 | 341                 |

Solution treated at 1,800° F. and aged at 1,825° F.

titanium content up to 3% may be effected without impairing its rupture ductility, while at the same time increasing room temperature hardness and tensile strength. It will be noted that we can obtain higher yield and tensile strengths (by the use of our permissible higher range of titanium) without adversely affecting rupture ductility due to the controlled vanadium additions. That is, our controlled vanadium additions permit the use of a higher titanium content without seriously increasing notch sensi-

tivity. This is true even when hardness is in excess of 290 Brinell which is in contradiction to alloy B. In this connection, attention is called to the data set forth in Table IV and Figure 3. Although, both the manganese and the vanadium contribute individually to good rupture ductility, they tend to decrease strength. A too high amount of manganese would decrease rupture strength greatly. However, the controlled amount of molybdenum increases the rupture strength. Thus, we add somewhat small amounts of vanadium, keep the manganese at about 1.0 to 2.0% (1.5% optimum) and the molybdenum at about 1.0 to 1.5% (1.25% optimum) to obtain both good rupture strength and ductility. In this connec-

tion, see the data of Table V, wherein melts A-286, A-373 and A-374 represent data on our alloys as compared to alloys having no molybdenum and vanadium or vanadium without molybdenum. It will be noted that melts A-56 and A-57 have a high manganese content and that melt A-54 has a lower content.

TABLE V

| Melt  | C   | Mn   | Si  | Cr   | Ni   | Ti  | Mo  | V   | Al  | Stress-Rupture at 1,200° F.—60,000 p. s. i. |                |                   |
|-------|-----|------|-----|------|------|-----|-----|-----|-----|---------------------------------------------|----------------|-------------------|
|       |     |      |     |      |      |     |     |     |     | Hrs. to Rupture                             | Percent Elong. | Percent Red. Area |
| A-54  | .05 | 1.3  | .73 | 14.2 | 25.2 | 1.8 | —   | .32 | .29 | 22                                          | 6.0            | 9.0               |
| A-286 | .04 | 1.3  | .82 | 14.4 | 26.1 | 1.8 | 1.3 | .32 | .03 | 15                                          | 5.7            | 10.4              |
| A-373 | .05 | 1.3  | .76 | 14.8 | 26.3 | 1.9 | 1.3 | .35 | .14 | 92                                          | 8.8            | 16.6              |
| A-374 | .04 | 1.14 | .78 | 14.9 | 26.5 | 1.7 | 1.3 | .34 | .16 | 211                                         | 10.6           | 22.2              |
| A-56  | .05 | 2.1  | .59 | 14.4 | 25.3 | 1.8 | —   | —   | .81 | 105                                         | 10.0           | 17.5              |
| A-57  | .04 | 4.9  | .54 | 14.2 | 25.4 | 1.6 | —   | —   | .30 | 39                                          | 7.8            | 18.0              |
|       |     |      |     |      |      |     |     |     |     | 4                                           | 13.5           | 15.2              |

High aluminum content has a similar effect as manganese in that it increases rupture ductility at the expense of rupture strength, even in the presence of molybdenum. This can be counteracted and the rupture strength greatly increased by the addition of cobalt as shown in Table VI.

In Figure 1, we have graphically shown the effect of the temperature of solution treatment of our alloy, based on standard and V-notch rupture strength and rupture ductility test data taken at 1200° F. and using 60,000 p. s. i.

In Figure 2 of the drawings, we have shown graphically the effect of titanium content on

TABLE VI

Effect of aluminum and cobalt

| Melt  | C   | Mn   | Si  | Cr   | Ni   | Ti  | Mo  | V   | Al  | Co   | Stress-Rupture at 1,200° F.—60,000 p. s. i. |                 |             |                   |
|-------|-----|------|-----|------|------|-----|-----|-----|-----|------|---------------------------------------------|-----------------|-------------|-------------------|
|       |     |      |     |      |      |     |     |     |     |      | Type Test                                   | Hrs. to Rupture | Percent El. | Percent Red. Area |
| A-416 | .04 | 1.16 | .63 | 14.7 | 26.0 | 1.8 | 1.3 | .27 | 3.1 | 20.1 | Std.                                        | 13              | 30.7        | 66.6              |
| A-409 | .04 | 1.11 | .85 | 14.8 | 26.1 | 1.7 | 1.2 | .32 | 1.1 | —    | Std.                                        | 491             | 8.6         | 15.7              |
| A-409 |     |      |     |      |      |     |     |     |     |      | V-notch                                     | 681             | —           | —                 |

It will be noted that the V-notch test of melt A-409 shows a life of 681 hours which indicates that cobalt added (within the specified range) to our alloy does not make it notch sensitive.

In Figure 3 of the drawings, we have shown graphically a comparison of V-notch rupture life and Standard test rupture life of alloys of our invention with various titanium contents as expressed in Brinell hardness when fully heat treated. The data as to our alloys is taken from Table IV. As compared to the patent disclosure of alloy B, where it is said that notch rupture strength is much lower than regular rupture strength once the hardness goes above about 290 Brinell, this graph shows that the V-notch rupture strength of our alloy is higher than the regular rupture strength all the way up to 341 Brinell. A comparison of the curves of Figures 2 and 3 and Table IV discloses that our alloy has a rupture elongation of about 10% at a hardness of 341 Brinell, as contrasted to .5% of alloy B at the same Brinell.

In our melts, commercial scavengers and de-oxidizers, such as calcium-silicon-manganese, calcium-silicon, silicon-zirconium, Grinal (titanium-aluminum-vanadium), Lan Cer Amp (about 50% lanthanum, 30% cerium and 20% rare earth metals) and L-Metal (about the same composition as Lan Cer Amp), have been used with advantage.

An alloy of our invention is particularly characterized by its ability to develop high strength

| Melt  | C   | Mn   | Si  | Cr   | Ni   | Ti  | Mo  | V   | Al  | Co   |
|-------|-----|------|-----|------|------|-----|-----|-----|-----|------|
| A-424 | .02 | 1.32 | .74 | 15.0 | 26.1 | 2.9 | 1.3 | .38 | .17 | —    |
| A-425 | .05 | 1.23 | .89 | 15.1 | 24.7 | 3.1 | 1.2 | .31 | .18 | 19.6 |

| Melt  | Stress-Rupture at 1,200° F.—60,000 p. s. i. |                |                   | Stress-Rupture at 1,350° F.—42,500 p. s. i. |                |                   |
|-------|---------------------------------------------|----------------|-------------------|---------------------------------------------|----------------|-------------------|
|       | Hrs. to Rupture                             | Percent Elong. | Percent Red. Area | Hrs. to Rupture                             | Percent Elong. | Percent Red. Area |
| A-424 | 301                                         | 7.5            | (1)               | 318                                         | 16.3           | 28.3              |
| A-425 | 1,361+                                      | (1)            | 11.0              | 769                                         | 11.0           | 19.3              |

<sup>1</sup> Test in progress.

properties (in its heat-treated state) up to 1350° F. with an inherently good rupture ductility and notch rupture strength. That is, the alloying elements of an alloy of our invention are so proportioned as to give it a high rupture ductility and strength at operating temperatures up to 1350° F. and a good ductility within the normally brittle range of 1000° to 1200° F. Such alloy is of an austenitic, ferrous-metal-containing type, such that the remainder is iron or substantially all iron with incidental impurities. For example, production melts may contain impurities such as sulphur, phosphorus, selenium, nitrogen, copper, zirconium, cerium, and lanthanum.

What we claim is:

1. A commercially producible and forgeable austenitic alloy steel suitable for moving part usage and having an inherently good rupture ductility with a high notch rupture strength at elevated temperatures of about 1000 to 1300° F., in which manganese, chromium, nickel, titanium, molybdenum and vanadium are the only essential elements, are critical within the ranges specified, and the specified contents of the elements manganese and vanadium are essentially in solid solution form in the alloy, and in which aluminum may be present in incidental amounts and up to about 2.50% with the presence of cobalt of up to about 25%; the composition consisting of carbon in a relatively small amount up to a maximum of about .15%, about .50 to 3.00% manganese, up to about 1.50% silicon, about 5 to 22% chromium, about 7 to 50% nickel, about .50 to 3.50% titanium, about .25 to 2.00% molybdenum, about .10 to 1.50% vanadium, and the remainder iron with incidental impurities.

2. An improved alloy as defined in claim 1, as further characterized by its fully developed properties when solution treated for about one hour at and quenched from about 1800° F., followed by age hardening for about 16 hours at and quenched from about 1325° F.

3. A commercially producible and forgeable austenitic alloy steel suitable for moving part usage and having an inherently good rupture ductility with a high notch rupture strength at elevated temperatures of about 1000 to 1300° F., in which manganese, chromium, nickel, titanium, molybdenum and vanadium are the only essential elements and the specified contents of the elements manganese and vanadium are essentially in solid solution form and in which aluminum may be present in incidental amounts from the addition of ferro-alloys; and the composition consisting of carbon in a relatively small amount up to a maximum of about .15%, about .50 to 3.00% manganese, up to about 1.50% silicon, about 5 to 22% chromium, about 7 to 50% nickel, about .50 to 3.50% titanium, about .25 to 2.00% molybdenum, about .10 to 1.50% vanadium, and the remainder iron with incidental impurities.

4. A commercially producible and forgeable austenitic alloy steel suitable for moving part usage and having an inherently good rupture ductility with a high notch rupture strength at elevated temperatures of about 1000 to 1300° F., in which manganese, chromium, nickel, titanium, molybdenum and vanadium are the only essential elements and the specified contents of the elements manganese and vanadium are essentially in solid solution form, and in which aluminum may be present up to about .40%; the composition consisting of carbon in a relatively small amount up to a maximum of about .15%, about .50 to 3.00% manganese, up to about 1.50% silicon, about 5 to 22% chromium, about 7 to 50% nickel, about .50 to 3.50% titanium, about .25 to 2.00% molybdenum, about .10 to 1.50% vanadium, and the remainder iron with incidental impurities.

con, about 5 to 22% chromium, about 7 to 50% nickel, about 1.50 to 3.50% titanium, about .50 to 1.50% molybdenum, about .10 to 1.50% vanadium, and the remainder iron with incidental impurities.

5. A commercially producible and forgeable austenitic alloy steel suitable for moving part usage and having an inherently good rupture ductility with a high notch rupture strength at elevated temperatures of about 1000 to 1300° F., in which manganese, chromium, nickel, titanium, molybdenum and vanadium are the only essential elements and the specified contents of the elements manganese and vanadium are essentially in solid solution form, and in which aluminum may be present in a maximum amount of about .40%; the composition consisting of carbon in a relatively small amount up to a maximum of about .15%, about .50 to 2.00% manganese, about .40 to 1.50% silicon, about 12 to 18% chromium, about 20 to 35% nickel, about 1.50 to 2.90% titanium, about 1 to 1.50% molybdenum, about .10 to .50% vanadium, and the remainder iron with incidental impurities.

10 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 99

13

2.5% titanium, about .50 to 1.50% molybdenum, about .10 to .70% vanadium, about 1 to 3.50% aluminum, about 19 to 25% cobalt, and the remainder iron with incidental impurities.

GUNTHER MOHLING.  
WASIL W. DYRKACZ.

References Cited in the file of this patent

## UNITED STATES PATENTS

| Number    | Name       | Date         |
|-----------|------------|--------------|
| 2,043,533 | Harrington | June 9, 1936 |

5

| Number    |
|-----------|
| 2,048,164 |
| 2,432,615 |
| 2,432,619 |

| Number  |
|---------|
| 929,727 |

10

14

| Name    | Date          |
|---------|---------------|
| Pilling | July 21, 1936 |
| Franks  | Dec. 16, 1947 |
| Franks  | Dec. 16, 1947 |

## FOREIGN PATENTS

| Country | Date         |
|---------|--------------|
| France  | Jan. 6, 1948 |